

May 20, 1924.

1,494,479

J. H. HASTE

PHOTOGRAPHIC FILM WITH LAMINATED SUPPORT HAVING INCREASED FLEXIBILITY

Filed Dec. 26, 1922



INVENTOR  
James H. Haste,  
BY R. L. Strichfield

ATTORNEY

Patented May 20, 1924.

1,494,479

# UNITED STATES PATENT OFFICE.

JAMES H. HASTE, OF ROCHESTER, NEW YORK, ASSIGNOR TO EASTMAN KODAK COMPANY, OF ROCHESTER, NEW YORK, A CORPORATION OF NEW YORK.

PHOTOGRAPHIC FILM WITH LAMINATED SUPPORT HAVING INCREASED FLEXIBILITY.

Application filed December 26, 1922. Serial No. 609,123.

*To all whom it may concern:*

Be it known that I, JAMES H. HASTE, a citizen of the United States of America, residing at Rochester, in the county of Monroe 5 and State of New York, have invented certain new and useful Improvements in Photographic Films with Laminated Supports Having Increased Flexibility, of which the following is a full, clear, and exact specification.

This invention relates to photographic film, the support of which is laminated. One object of the invention is to provide a film, the flexibility of which will be increased both in degree and permanence without impairing other desirable qualities. Other objects will hereinafter appear.

The single figure in the drawing shows a diagrammatic sectional view of one embodiment of my invention on an exaggerated scale.

When attempts are made to increase the flexibility of photographic films by increasing the amounts of customary flexibility-inducing substances in the compositions of the support, limits are quickly reached because other qualities, such as strength, hardness, transparency and the like may be impaired before the desired degree of flexibility is obtained. It has now been found that when the support is composed of compositions based chiefly upon cellulosic addition compounds, such as cellulose acetate, cellulose ether and nitrocellulose, the flexibility 25 is affected to an unusual degree by very small amounts of moisture regardless of other flexibility-inducing substances. Quantities of moisture, which are not detectable by touch but only by careful analytical 30 methods greatly alter the suppleness and flexibility of the film.

I have discovered that the benefits due to small amounts of moisture may be obtained in a very durable form by creating a localized reservoir of moisture within the film, rather than by initially distributing the entire reserve of moisture throughout the body of the film. In other words, I find that the 45 flexibility of the film may be increased by providing a laminated support, the layers of which are interunited in a zone which contains a reserve of moisture.

In the drawing, 1 indicates any suitable photographically sensitive layer, say, for instance, a coating of gelatino-silver haloid

emulsion. Layers 2, which constitute the support, are composed of addition compounds such as cellulose acetate, cellulose ether, and nitrocellulose. Since cellulose acetate gives the most marked results when 60 the reservoir of moisture-carrying material of my invention is employed, I use it in the preferred form of my invention, but the principle is very useful also in connection with laminated cellulose ether and nitrocellulose 65 films. At 3 I have indicated the zone of interunion in which the entire adjacent faces of the laminations are blended or welded together by a cement. Because of the lack of a sharp line of demarcation, solid 70 lines have been omitted from the boundaries of this layer 3.

The compositions of the layers 2 may be those usually employed for the manufacture 75 of flexible films. These layers, say of cellulose acetate, are welded or cemented by hand or by any usual apparatus for uniting sheet materials of this kind. The following cement illustrates one that is suitable for forming my moisture reservoir, — $\frac{1}{2}$  parts of glycerin 80 mixed with a bath of 20 parts acetone, 20 parts methyl alcohol, 40 parts methyl acetate, 19 parts butyl acetate, and a trace of cellulosic material addition compound, say, for instance, 1 part of nitrocellulose. The 85 glycerin preferably has moisture absorbed in it before it is mixed in the cement but it may absorb the moisture later.

The zone or layer of interunion 3, thus produced, contains the moisture-carrying 90 substance of the cement, of which glycerin is the preferred example, and thereby possesses a reserve of moisture. If the layers 2 tend to become too dry, especially in an arid climate, the moisture from this reserve works 95 its way out from zone 3 into said layers and maintains their flexibility to a degree that is strikingly useful. The above formula is also applicable to nitrocellulose films. When cellulose ethers are employed, it may be 100 modified by using other solvents, such as ethyl alcohol or chloroform in place of methyl alcohol and acetone.

Having thus described my invention, what I claim as new and desire to secure by Letters Patent is:

1. As an article of manufacture, a photographic film comprising a photographically sensitive layer and a laminated flexible light-transmitting support therefor, said support 110

including a plurality of layers of cellulosic addition compounds, the flexibility of which compounds is enhanced by moisture, said layers being interunited throughout their adjacent faces and each zone of interunion containing moisture-carrying material.

2. As an article of manufacture, a photographic film comprising a photographically sensitive layer and a laminated flexible transparent support therefor, including two layers of cellulose acetate united by a com-

position containing a hygroscopic substance to increase the flexibility of said support.

3. As an article of manufacture, a photographic film comprising a photographically sensitive layer and a support therefor, including two layers of cellulose acetate united by a composition containing glycerin.

Signed at Rochester, New York, this 16th day of December, 1922.

JAMES H. HASTE.